

## [54] METAL ELECTRODES AND COATINGS THEREOF

[75] Inventors: **Louis Degueldre; Yves Gobillon**, both of Brussels; **Lucien Clerbois, Vilvoorde; Louis Bourgeois**, Brussels, all of Belgium

[73] Assignee: **Solvay & Cie**, Brussels, Belgium

[22] Filed: **July 29, 1971**

[21] Appl. No.: **167,164**

## [30] Foreign Application Priority Data

July 29, 1970 Luxembourg ..... 61433

[52] U.S. Cl. ..... **204/290 F**, 136/120 FC, 204/98, 423/594, 423/595, 423/599, 423/600

[51] Int. Cl. ..... **B01k 3/06**, C01b 11/26

[58] Field of Search ..... 204/290 F, 291; 136/120 FC; 423/593, 594, 599, 600

## [56]

## References Cited

## UNITED STATES PATENTS

|           |         |                    |           |
|-----------|---------|--------------------|-----------|
| 3,070,422 | 12/1962 | Bayer .....        | 423/595   |
| 3,103,484 | 9/1963  | Messner .....      | 204/290 F |
| 3,329,594 | 7/1967  | Anthony et al..... | 204/290 F |
| 3,449,064 | 6/1969  | Bayer .....        | 423/593   |
| 3,607,416 | 9/1971  | Sizer, Sr. ....    | 204/290 F |
| 3,616,446 | 10/1971 | De Witt.....       | 204/290 F |
| 3,691,052 | 9/1972  | Langley .....      | 204/290 F |

Primary Examiner—F. C. Edmundson  
Attorney, Agent, or Firm—Spencer & Kaye

## [57]

## ABSTRACT

An electrode coating having the formula  $A_2BO_6$ , where A represents trivalent elements having anionic radius comprised between 0.50 and 0.73 Angstrom and where B represents hexavalent elements having an ionic radius comprised between 0.50 and 0.70.

8 Claims, 2 Drawing Figures



PATENTED OCT 1 1974

3,839,181



FIG. 1



FIG. 2

## METAL ELECTRODES AND COATINGS THEREOF

## BACKGROUND OF THE INVENTION

The present invention relates to a new type of coating serving as the operative surface of an electrode.

## SUMMARY OF THE INVENTION

The present invention concerns a new coating for metal electrodes. The coating comprises a compound having  $A_2BO_6$  as its general formula, where A represents one or more elements of valence 3, having an ionic radius comprised between 0.50 and 0.73 Angstrom, and B represents one or more elements of valence 6, having an ionic radius comprised between 0.50 and 0.60 Angstrom. The symbol O stands as usual for oxygen.

The coating may be  $A_2BO_6$  alone or an addition compound of  $A_2BO_6$  with another stoichiometric compound having the formula  $MO_2$  or  $M'M''O_4$ , where M represents one or more elements of valence 4, selected from Ir, Mn, Os, Rh, Ru, Sn and Ti, M' represents one or more elements of valence 3 selected from Al, Cr, Fe, Ga and Rh, and M'' represents one or more elements of valence 5, selected from Nb, Sb, Ta and V.

Preferably, A represents one or more elements selected from Co, Fe, Cr, Mn, Al, Ga, Ir, Rh and V, while B represents one or more elements selected from Te, W, Mo and Re.

## BRIEF DESCRIPTION OF THE DRAWING

FIG. 1 is an elevational view of a coated electrode according to the invention.

FIG. 2 is a cross sectional view from the line II-II of FIG. 1.

## DESCRIPTION OF THE PREFERRED EMBODIMENTS

Referring firstly to FIGS. 1 and 2, a conductive coating 11, such as  $Rh_2WO_6$ , is shown placed on a strip of metal 12, such as titanium.

It is preferred to place the conductive coating of the present invention on a metal support at least superficially made of titanium or a titanium metal. Advantageously, titanium is clad on a core of a more conductive metal such as copper, aluminum, iron, or alloys of these metals.

Preferably, the coating of the present invention consists, essentially of the compounds as set forth in the appended claims; yet more preferably, the coating consists of those compounds.

Electrodes provided with catalytic coatings according to the invention can be used for different electrochemical processes, such as cathodic protection, desalination or purification of water, water or hydrochloric acid electrolysis, electric current production in fuel cells, reduction or oxydation processes of organic compounds or electrolytic manufacture of peroxide salts but they are particularly useful as anodes for the electrolysis of aqueous solutions of alkali metal halides, especially sodium chloride, in diaphragm cells as well as in mercury-cathode cells, where they catalyse the discharge of chloride ions according to the half reaction  $2Cl^- \rightarrow Cl_2 + 2e^-$  under a remarkably low overvoltage which remains substantially unvaried over an electrode lifetime. Under the conditions ruling in these cells, the anode wear is very slow, thus providing practically un-

limited lifetime and avoiding the need for cell opening and coating restoration.

Further illustrative of the present invention are the following examples. All concentrations are given on a solution basis, unless indicated otherwise. Thus, for example, a solution of 0.45 g-at W/l means that there are 0.45 gram-atoms of tungsten in one liter of solution. Example 1:

$A_2BO_6$  (alone), where A = Rh and B = W.

Dihydrated rhodium nitrate,  $Rh(NO_3)_3 \cdot 2H_2O$ , and tungsten chloride,  $WCl_6$ , were separately dissolved at room temperature in N,N-dimethyl formamide (DMF),  $HCON(CH_3)_2$ , to give concentrations of 0.1 gram-atoms Rh/liter of solution and 0.46 gram-atoms W/liter of solution, respectively. These two solutions were then mixed in suitable proportions to give a Rh/W atom ratio of 2/1.

Several coats of this composition were painted onto titanium strips which had been degreased in hot trichloroethylene and immersed for 4-5 hours at about 90°C in an aqueous solution of 10 percent oxalic acid to etch the surface. For painting, titanium strips were placed on a heating plate at 100°-125°C. After each coating, the strips were heated for 15 minutes at from 300° to 450°C. After the fifth coating, the coated strips were heated in a furnace at 475°C for 5 hours. The coating thus obtained was analyzed and found to contain the compound  $Rh_2WO_6$ . It was present in an amount equal to approximately 5 grams per square meter of the titanium surface. It adhered tightly to the underlying titanium support and passed successfully a test consisting of attempting to tear off the coating with an adhesive tape applied under pressure.

The thus-coated titanium strips were subjected, as anodes, to two different tests: the first one to measure the overvoltage for the liberation of chlorine under a given anodic current density (10 kA/m<sup>2</sup>), the second one to determine the wear or consumption of noble metal as related to the quantity of evolved chlorine. The term "overvoltage" is used herein in the same sense as it is used at pages 488-492 of "Physical Chemistry" by Walter J. Moore, Prentice-Hall Inc., Second Edition.

In the overvoltage test, the coated strips were used as anodes for the electrolysis of a brine containing 250 g NaCl/kg. of solution saturated with chlorine at 60°C and at an approximate pH of 2. Under these conditions, the coated strips of this example showed an overvoltage in the range 170-260 mV under an anodic current density of 10 kA/m<sup>2</sup>.

In the wear test, the coated strips were used as anodes in a cell with a flowing mercury cathode for the electrolysis of a brine saturated with sodium chloride and chlorine, between 80° and 85°C, under a constant anode-cathode potential difference, the test being stopped when the current density was reduced to one half of its initial value (initial value generally was between 30 and 40 kA/m<sup>2</sup>). Under these conditions, the tested strips produced 9 tons of chlorine per square meter of active surface; the rhodium consumption lay below 500 mg per ton of chlorine produced under an average current density of 20 kA/m<sup>2</sup>.

Example 2:

$A_2BO_6$  (alone), where A = Rh and B = Te.

The 0.1 gram-atoms/1 Rh solution used in Example

1 was mixed with a solution of  $\text{TeO}_2$  in 12 N hydrochloric acid to give an Rh/Te atom ratio of 2.

Five coats of this composition were applied onto titanium strips under the same conditions as in Example 1. The coating thus obtained was analyzed and found to contain the compound  $\text{Rh}_2\text{TeO}_6$ . It was present in an amount of approximately 5 g/m<sup>2</sup> and showed a very good adhesion during the tearing off tests.

In an overvoltage test carried out under the same conditions as in Example 1, the thus-coated strips showed an overvoltage in the range 315-430 mV, under an anodic current density of 10 kA/m<sup>2</sup>.

In a wear test, also carried out under the conditions of Example 1, these same coated strips produced 15 tons  $\text{Cl}_2/\text{m}^2$  under an average anodic current density of 20 kA/m<sup>2</sup>, the Rh wear being in the range of 200 mg/ton  $\text{Cl}_2$ .

Example 3:

$\text{A}_2\text{BO}_6$  (alone), where  $A = \text{Rh}$  and  $B = 1/3 \text{ Te} + 2/3 \text{ W}$ .

Hydrated rhodium trichloride and tungsten chloride  $\text{WC1}_6$  were separately dissolved in DMF. 0.166 ml of the W solution containing 0.49 g-at W/l and 6.5 mg of tellurium oxide,  $\text{TeO}_2$ , previously dissolved in 0.1 ml concentrated hydrochloric acid were added to 10 ml of the Rh solution containing 0.0245 g-at Rh/l.

Four coats of this mixture were applied at room temperature onto titanium strips. The strips were dried in air for 30 minutes and heated at 350°C for 15 minutes, after each coating. They were finally heated in a furnace at 500°C for 66 hours.

The thus obtained  $\text{Rh}_2(\text{Te}_{1/3}\text{W}_{2/3})\text{O}_6$  coating was present in an amount near to 7 g/m<sup>2</sup>; the coating showed an excellent adhesion.

In an overvoltage test carried out under the same conditions as in Example 1, the thus coated strips showed an average overvoltage of 350 mV under a current density of 10 kA/m<sup>2</sup>.

Example 4:

$\text{A}_2\text{BO}_6$  (alone), where  $A = 0.9 \text{ Rh} + 0.1 \text{ Fe}$  and  $B = \text{W}$ .

0.053 ml of a solution of  $\text{FeCl}_3 \cdot 6\text{H}_2\text{O}$  in DMF at 0.51 g-at Fe/l and 0.28 ml of the tungsten solution of Example 3 were added to 10 ml of the rhodium solution used in Example 3. a. seven coats of this composition were applied at room temperature onto titanium strips. The strips were dried in the air and heated for 15 minutes at 350°C after each application. Upon final firing at 500°C for 20 hours, a coating of 9 g/m<sup>2</sup> ( $\text{Rh}_{0.9}\text{Fe}_{0.1}\text{W}_2\text{O}_6$ ) was obtained which showed a good adhesion. In an overvoltage test carried out under the same conditions as in Example 1, the thus coated strips showed an average overvoltage of 290 mV under a current density of 10 kA/m<sup>2</sup>. b. The same coating was prepared, but only four coats of the said composition were applied onto the titanium strips disposed on a heating plate. After each coating, the strips were heated in the range 350°-425°C. They were finally fired at 500°C for 17 hours. The average deposit weight of the thus obtained ( $\text{Rh}_{0.9}\text{Fe}_{0.1}\text{W}_2\text{O}_6$ ) coating was 6.7 g/m<sup>2</sup>. The thus coated strips showed better adhesion to the support than strips obtained by applying the same coating composition at room temperature.

In an overvoltage test carried out under the same conditions as in Example 1, the thus coated strips

showed overvoltages between 260 and 360 mV under a current density of 10 kA/m<sup>2</sup>.

Example 5:

5 Addition compound  $\text{A}_2\text{BO}_6 + 3\text{MO}_2$ , where  $A = \text{Cr}$ ,  $B = \text{W}$  and  $M = \text{Ru}$ .

Tungsten chloride,  $\text{WCl}_6$ ,  $\text{CrCl}_3 \cdot 6\text{H}_2\text{O}$ , and hydrated  $\text{RuCl}_3$  were dissolved separately in DMF to give solutions of 0.45 g-at W/l, 0.46 g-at Cr/l and 0.5 g-at Ru/l respectively, which were mixed in suitable proportions in order to give a Ru/Cr/W atom ratio of 3/2/1.

10 Five coats of the said composition were applied onto titanium strips under the same conditions as in Example 1. After firing, a coating of  $\text{Cr}_2\text{WO}_6 + 3\text{RuO}_2$  was obtained. The adhesion of this coating to the support was not perfect.

Nevertheless, used as anodes under the same conditions as in Example 1, the thus coated strips also presented very interesting electrochemical properties.

20 Example 6:

Addition compound  $\text{A}_2\text{BO}_6 + 3\text{MO}_2$ , where  $A = \text{Fe}$ ,  $B = \text{W}$  and  $M = \text{Ru}$ .

The 0.51 g-at Fe/l solution of Example 4 and the solutions of 0.46 g-at Cr/l and 0.5 g-at Ru/l of Example 25 5 were mixed together in suitable proportions to give a Ru/Fe/W atom ratio of 3/2/1.

30 Five coats of the resulting mixtures were applied onto titanium strips under the same conditions as in Example 1, and after firing, a coating of  $\text{Fe}_2\text{WO}_6 + 3\text{RuO}_2$  was obtained. This coating showed relatively poor adhesion to the support, but interesting anodic polarization properties in chlorinated brine.

Example 7:

35 Addition compound  $\text{A}_2\text{BO}_6 + 3\text{MO}_2$ , where  $A = \text{Cr}$ ,  $B = \text{Te}$  and  $M = \text{Ru}$ .

The solutions of Cr and Ru mentioned in Example 5 were mixed in a proper proportion and a suitable 40 amount of  $\text{TeO}_2$  dissolved in 12 N HCl was added in order to obtain a Ru/Cr/Te atom ratio of 3/2/1.

45 Applied onto titanium strips under the conditions described in Example 1, this composition gave, after firing, a coating of  $\text{Cr}_2\text{TeO}_6 + 3\text{RuO}_2$  whose adhesion to the support was satisfactory and which showed interesting anodic polarization properties in chlorinated brine.

Example 8:

50 Addition compound  $\text{A}_2\text{BO}_6 + 3\text{MO}_2$ , where  $A = \text{Rh}$ ,  $B = \text{Te}$  and  $M = \text{Ru}$ .

A solution A containing 0.2 g-at Ru/l was prepared. First, ruthenium chloride,  $\text{RuCl}_3 \cdot x \text{H}_2\text{O}$  was dissolved in a quantity of ethanol, then chloroform was added in an amount equal to the volume of the ethanol solution and finally turpentine *a* (boiling point above 150°C), previously sulphurated to 20 percent through reflux heating of 80 g turpentine *a* with 20 g sulphur for 3 hours, was added, also in an amount equal to the volume of the 55 ethanol solution.

60 By operating in the same way with rhodium chloride,  $\text{RhCl}_3 \cdot x \text{H}_2\text{O}$ , a solution B containing 0.2 g-at Rh/l was prepared.

A solution C of 0.2 g-at Te/l was prepared by dissolving tellurium chloride,  $\text{TeCl}_4$ , (resulting from the action of chlorine upon tellurium) in two volumes of ethanol, to which five volumes of turpentine *a* sulphu-

rated to 40 percent were then added, the whole being heated on a water-bath until the formed precipitate had completely disappeared.

Then, a solution D was prepared by mixing 1 volume of ethanol, one volume of chloroform and 1 volume of turpentine a.

Finally, mixing 3 ml of solution A,  
2 ml of solution B,  
1 ml of solution C, and  
14 ml of solution D,

a mixture was obtained which was applied onto titanium strips previously degreased and etched as described in Example 1.

This coating was carried out in the air at room temperature. After each coating, the strips were heated for 15 minutes at 500°C.

After application of 10 coatings in accordance with the aforesaid conditions, the strips were finally fired at 500°C for 5 hours in the presence of air.

The deposit weight of the thus obtained coating of  $\text{Rh}_2\text{TeO}_6 + 3\text{RuO}_2$  was approximately 4 g/m² and its adhesion to the support was acceptable.

In an overvoltage test carried out under the same conditions as indicated in Example 1, the thus coated strips showed an overvoltage of 245 mV under an anodic current density of 10 kA/m².

In a wear test, also carried out as indicated in Example 1, these coated strips produced 120 tons of chlorine/m² working continuously under an average current density of 24 kA/m². The consumption of noble metal was under 20 mg Rh + Ru per ton of produced chlorine.

Example 9:

Addition compound  $\text{A}_2\text{BO}_6 + 12\text{ MO}_2$ , where  $A = \text{Rh}$ ,  $B = \text{Te}$  and  $M = \text{Ru}$ .

By dissolving ruthenium chloride  $\text{RuCl}_3 \cdot x \text{H}_2\text{O}$  in n-pentanol, a solution A of one g-at Ru/l was prepared.

By operating in the same way with rhodium chloride  $\text{RhCl}_3 \cdot x \text{H}_2\text{O}$ , a solution B of 0.5 g-at Rh/l was prepared.

Then, a solution of allotelluric acid in ethanol of 0.5 g-at Te/l (solution C) was prepared. Allotelluric acid was obtained by keeping telluric acid,  $\text{H}_2\text{TeO}_4 \cdot 2\text{H}_2\text{O}$ , at 150°C for 90 minutes in a sealed tube.

Mixing 5 ml of solution A,  
1.7 ml of solution B,  
0.84 ml of solution C, and  
41.5 ml of n-pentanol,

a mixture was obtained which was applied onto titanium strips previously degreased and etched as in Example 1.

For the application of this mixture, the titanium strips were disposed, in the air, on a heating plate at approximately 100°C. After each application and evaporation of excess solvent, the coated strips were heated for 15 minutes at 350°C. After seven coatings had been applied under the same conditions, the coated strips were finally fired for one hour at 500°C in the presence of air.

The thus obtained coating of  $\text{Rh}_2\text{TeO}_6 + 12\text{ RuO}_2$  of about 5 g/m² adhered tightly to the support as shown by the test consisting of attempting to tear off the coating with an adhesive tape applied under pressure.

In an overvoltage test carried out as in Example 1, the thus coated strips showed an overvoltage of 95 mV under an anodic current density of 10 kA/m².

In a wear test carried out as in Example 1, the coated strips produced more than 82 tons of chlorine/m², working continuously under current densities between 36 and 25 kA/m². At this stage, the use limit was not reached and the wear test continued.

Example 10:

10 Addition compound  $\text{A}_2\text{BO}_6 + 6\text{MO}_2$ , where  $A = \text{Rh}$ ,  $B = \text{Te}$ , and  $M = \text{Ir}$ .

A solution of 0.019 g-at Ir/l (solution A) was prepared by dissolving chloro-iridic acid  $\text{H}_2\text{IrCl}_6 \cdot x\text{H}_2\text{O}$  in dimethyl sulphoxide (DMSO),  $\text{CH}_3\text{SOCH}_3$ .

A solution of 0.194 gram-atom Rh/l (solution B) was prepared by dissolving rhodium nitrate  $\text{Rh}(\text{NO}_3)_3$  in glycol,  $\text{HOCH}_2 - \text{CH}_2\text{OH}$ .

Finally, 25.2 mg  $\text{TeO}_2$  were substantially dissolved in a few drops of concentrated HCl (solution C).

Mixing 50 ml of solution A  
1.65 ml of solution B and  
the whole of solution C,  
a mixture was obtained which was applied onto titanium strips previously degreased and etched according to Example 1.

For the application of the mixture, the titanium strips were disposed, in the air, on a heating plate at about 100°C.

30 After each application, the coated strips were heated for 5 minutes at 400°C.

After 12 coatings had been applied under the same conditions, six further coatings were applied with intermediate heatings of 15 minutes at 440°C.

Finally, the coated strips were fired for 16 hours at 475°C in the presence of air.

The thus obtained coating of  $\text{Rh}_2\text{TeO}_6 + 6\text{IrO}_2$  (about 8 g/m²) passed successfully a test consisting of attempting to tear off the coating with an adhesive tape applied under pressure.

In an overvoltage test carried out as in Example 1, the thus coated strips showed an overvoltage of 135 mV under an anodic current density of 10 kA/m².

45 In a wear test carried out as in Example 1, these same coated strips produced more than 63 tons of chlorine per square meter of active anodic surface under an average current density of 24 kA/m². At this stage, the use limit was not yet reached and the wear test continued.

Example 11:

55 Addition compound  $2\text{A}_2\text{BO}_6 + 3\text{M}'\text{M}''\text{O}_4$ , where  $A = \text{Rh}$ ,  $B = \text{Te}$ ,  $M' = \text{Rh}$  and  $M'' = \text{Sb}$ .

Hydrated  $\text{RhCl}_3$  and  $\text{SbCl}_3$  were separately dissolved in n-hexanol to give solutions of 0.5 g-at Rh/l (solution A) and 1 g-at Sb/l (solution B) respectively.

5 ml of solution A,  
1.1 ml of solution B,  
1.4 ml of solution C of Example 9, and  
42.5 ml of n-hexanol were mixed.

60 Seven coatings of the mixture were applied onto titanium strips previously degreased and etched as in Example 1. For the application of the mixture, the strips were disposed on a heating plate at approximately 70°C. After each of an initial six applications, the strips were heated for 15 minutes at 500°C, whereas after the

seventh application, they were finally fired for 1 hour at 500°C.

The thus obtained coating of  $2\text{Rh}_2\text{TeO}_6 + 3\text{RhSbO}_4$  of  $2.6 \text{ g/m}^2$  passed successfully the test consisting of attempting to tear off the said coating with an adhesive tape applied under pressure.

In an overvoltage test carried out under the same conditions as in Example 1, the thus coated strips showed an overvoltage of 450 mV under an anodic current density of  $10 \text{ kA/m}^2$ .

The characteristics of the 11 examples as hereinbefore detailed are given in the following table.

| Example No. | Composition of the coating                             | Thickness in $\text{g/m}^2$ | Adhesion     | Overvoltage in mV at $10 \text{ kA/m}^2$ | Coating wear test                        |                                    |                                                                    |
|-------------|--------------------------------------------------------|-----------------------------|--------------|------------------------------------------|------------------------------------------|------------------------------------|--------------------------------------------------------------------|
|             |                                                        |                             |              |                                          | $\text{Cl}_2$ produced in $\text{t/m}^2$ | Current density in $\text{kA/m}^2$ | Consumption of noble metal in $\text{mg/t}$ produced $\text{Cl}_2$ |
| 1           | $\text{Rh}_2\text{WO}_6$                               | 5                           | excellent    | 170-260                                  | 9                                        | 20                                 | <500                                                               |
| 2           | $\text{Rh}_2\text{TeO}_6$                              | 5                           | very good    | 315-430                                  | 15                                       | 20                                 | 200                                                                |
| 3           | $\text{Rh}_2(\text{Te}_{1/3}\text{W}_{2/3})\text{O}_6$ | 7                           | excellent    | 350                                      |                                          |                                    |                                                                    |
| 4a          | $(\text{Rh}_{0.9}\text{Fe}_{0.1})_2\text{WO}_6$        | 9                           | good         | 290                                      |                                          |                                    |                                                                    |
| 4b          | do.                                                    | 6.7                         | very good    | 260-360                                  |                                          |                                    |                                                                    |
| 5           | $\text{Cr}_2\text{WO}_6.3\text{RuO}_2$                 | 5                           | poor         | interesting                              |                                          |                                    |                                                                    |
| 6           | $\text{Fe}_2\text{WO}_6.3\text{RuO}_2$                 |                             | do.          | do.                                      |                                          |                                    |                                                                    |
| 7           | $\text{Cr}_2\text{TeO}_6.3\text{RuO}_2$                |                             | satisfactory | do.                                      |                                          |                                    |                                                                    |
| 8           | $\text{Rh}_2\text{TeO}_6.3\text{RuO}_2$                | 3.7                         | do.          | 245                                      | 120                                      | 24                                 | <20                                                                |
| 9           | $\text{Rh}_2\text{TeO}_6.12\text{RuO}_2$               | 5                           | very good    | 95                                       | >82                                      | 36-25                              |                                                                    |
| 10          | $\text{Rh}_2\text{TeO}_6.6\text{IrO}_2$                | 8                           | do.          | 135                                      | >63                                      | 24                                 |                                                                    |
| 11          | $2\text{Rh}_2\text{TeO}_6.3\text{RhSbO}_4$             | 2.6                         | excellent    | 450                                      |                                          |                                    |                                                                    |

A coating which has "interesting overvoltage properties" is a coating for which an overvoltage of about 450 mV may be obtained in the test carried out with chlorinated brine. For industrial uses in electrolysis of  $\text{NaCl}$  brine for producing chlorine, 500 mV may be considered as the maximum overvoltage acceptable for economic view point. For other electrochemical processes such as cathodic protection and all the uses where Cr and Fe, particularly, are not subject to corrosion, 500 mV is not a critical factor, and so, these coatings may be interesting.

In the general formula  $\text{A}_2\text{BO}_6$ , A is an element at the valence 3 having an ionic radius comprised between 0.5 and 0.75 Angstrom and B is an element at the valence 6 having an ionic radius comprised between 0.5 and 0.6 Angstrom. Outside these ionic radius ranges, the compound  $\text{A}_2\text{BO}_6$  of the invention cannot be obtained. According to this restriction the elements may be chosen in the tables published by R. D. Shannon and C. T. Prewitt-Acta. Cryst. 1969, B 25, p. 925 - 946 and Acta. Cryst. 1970, B 26, p. 1046 - 1048.

Among all these elements, the more commonly available, i.e., Co, Cr, Fe, Mn, Al, Ga, Ir, Rh and V for A and Te, W, Mo and Re for B are preferred.

It will be understood that the above description and foregoing Examples of the present invention are susceptible of various modifications, changes and adaptations, and the same are intended to be comprehended within the meaning and range of equivalents of the appended claims.

We claim:

1. A metallic electrode having a conductive coating, said coating comprising a compound of the general formula  $\text{A}_2\text{BO}_6$ , wherein A represents at least one element at the valence 3, selected from the group consisting of Ir and Rh, and B represents at least one element at the valence 6, selected from the group consisting of Te, W, Mo and Re.

2. A metallic electrode having a conductive coating

as claimed in claim 1, wherein the said compound  $\text{A}_2\text{BO}_6$  is rhodium tungstate,  $\text{Rh}_2\text{WO}_6$ .

3. A metallic electrode having a conductive coating as claimed in claim 1, wherein the said compound  $\text{A}_2\text{BO}_6$  is rhodium tellurate,  $\text{Rh}_2\text{TeO}_6$ .

4. A metallic electrode having a conductive coating as claimed in claim 1, said conductive coating further comprising an oxide of  $\text{MO}_2$  type, where M represents at least one element at the valence 4 selected from the group consisting of Ir, Mn, Os, Rh, Ru, Sn, and Ti.

5. A metallic electrode having a conductive coating as claimed in claim 1, said conductive coating, further comprising an oxide of  $\text{M}'\text{M}''\text{O}_4$  type, where  $\text{M}'$  repre-

sents at least one element at the valence 3 selected from the group consisting of Al, Cr, Fe, Ga, and Rh, and  $\text{M}''$  represents at least one element at the valence 5 selected from the group consisting of Nb, Sb, Ta, and V.

6. A metallic electrode having a conductive coating as claimed in claim 1 wherein B is at least partially Te.

7. A metallic electrode having a conductive coating, said coating comprising a compound of the general formula  $\text{A}_2\text{BO}_6$ , wherein A represents at least one element at the valence 3 selected from the group consisting of Co, Cr, Fe, Mn, Al, Ga and V, and B represents at least one element at the valence 6 selected from the group consisting of Te, W, Mo and Re, the said conductive coating further comprising at least one other compound containing at least one element selected from the group consisting of Ir, Os, Rh and Ru, said other compound being selected from the group consisting of  $\text{MO}_2$  and  $\text{M}'\text{M}''\text{O}_4$  where:

M represents at least one element at the valence 4 selected from the group consisting of Ir, Mn, Os, Rh, Ru, Sn and Ti

$\text{M}'$  represents at least one element at the valence 3 selected from the group consisting of Al, Cr, Fe, Ga, and Rh

$\text{M}''$  represents at least one element at the valence 5 selected from the group consisting of Nb, Sb, Ta and V.

8. An electrode suitable for use in electrochemical processes, comprising a support at least superficially containing titanium and having anodic polarization properties comparable with those of titanium, and on at least a part of the surface of said support a conductive coating comprising a compound of general formula  $\text{A}_2\text{BO}_6$ , wherein A represents one or more elements at valence 3 selected from the group consisting of Co, Cr, Fe, Mn, Al, Ga and V, and B represents at least one element at the valence 6 selected from the group consisting of Te, W, Mo and Re.

\* \* \* \*